

# United States Patent [19]

Garth

[11] 3,925,030  
[45] Dec. 9, 1975

[54] ANTI-ICING COMPOSITION

[75] Inventor: Bruce Hollis Garth, Newark, Del.

[73] Assignee: E. I. Du Pont de Nemours & Co.,  
Wilmington, Del.

[22] Filed: Oct. 6, 1972

[21] Appl. No.: 295,660

[52] U.S. Cl. .... 44/56; 44/56 D; 44/66;  
44/70; 44/77

[51] Int. Cl.<sup>2</sup> .... C10L 1/02

[58] Field of Search .... 44/DIG. 1, 66, 70, 77

[56] References Cited

UNITED STATES PATENTS

|           |        |                |           |
|-----------|--------|----------------|-----------|
| 2,632,695 | 3/1953 | Landis et al.  | 44/66     |
| 2,786,745 | 3/1957 | Stayner et al. | 44/DIG. 1 |
| 2,807,526 | 9/1957 | Foreman        | 44/DIG. 1 |
| 2,952,121 | 9/1960 | Mitacek        | 44/DIG. 1 |
| 3,032,971 | 3/1962 | Shotton        | 44/DIG. 1 |

3,270,497 9/1966 Malick ..... 44/77  
3,416,902 12/1968 Anderson et al. ..... 44/DIG. 1

Primary Examiner—Daniel E. Wyman

Assistant Examiner—Y. Harris Smith

[57] ABSTRACT

An anti-icing composition, useful as a gasoline additive, comprising 30–90 weight % of a gasoline soluble organic compound of the formula Z—OH and 10–70 weight % of a gasoline soluble polycarboxy hydrocarbon having 25–75 carbon atoms and at least ten carbon atoms per carboxy group, Z containing about 4–180 carbon atoms and being selected from aliphatic hydrocarbyl, hydroxyaliphatic hydrocarbyl, hydro-poly(oxyalkylene), alkyl poly(oxyalkylene) and alkyl-phenyl poly(oxyalkylene), for example, an anti-icing composition comprising 30–90 weight % of linoleic acid dimertrimer acid and 10–70 weight % of dipropylene glycol.

14 Claims, 1 Drawing Figure





## ANTI-ICING COMPOSITION

## BACKGROUND OF THE INVENTION

## 1. Field of the Invention

This invention relates to gasoline additives which provide carburetor anti-icing protection.

## 2. Description of the Prior Art

Carburetted internal combustion engines have a tendency to stall during cool wet weather, particularly when they are run at idling speeds before being sufficiently warmed up. The formation of ice in the fuel lines and in the carburetor, particularly on the throttle plate and its adjacent walls, is generally recognized as the cause of such engine stalling. Carburetor icing generally occurs most readily when the atmospheric temperature is about 22°-50°F., the relative humidity is greater than 65% and the fuel is highly volatile (ASTM Method D-86 distillation of less than about 300°F.). Although stalling due to carburetor icing is a temporary phenomenon, such stalling usually being eliminated when the engine is thoroughly warm, it is nevertheless undesirable because of the inconvenience, driving annoyance and safety hazard. To prevent or minimize carburetor icing, changes in the carburetor design and/or rapid means of warming the carburetor may be useful but it is generally recognized that the most effective means of solving the problem is by the use of proper anti-icing additives in the fuel.

Anti-icing additives known in the art include, in addition to the commonly known lower molecular weight alkanols such as methanol, ethanol and isopropanol, other alcohols such as tetrahydrofurfuryl alcohol, polyalkylene glycols, mixtures of glycol ethers, polyalkylene glycol monoethers, alkanolamines, polyamines, amides, amine carboxylate salts, a mono- and/or dialkyl phosphate at least partially neutralized with an amine, and combinations such as an alcohol and an ether, benzoic acid and an aminoglycol ether, glycerine and a glycol ether, an N-alkylpyrrolidone and an alkylene diol and a polyhydroxy compound and an aminoamide.

Known anti-icing agents may be deficient for one or more of the following reasons:

1. Most anti-icing additives, and particularly the water soluble additives which function primarily as antifreeze for the fuel, must be used in such high concentrations (up to about 1 weight %) as to make commercial use uneconomical.

2. Many anti-icing additives promote a high degree of fuel/water interaction, the additive either being readily extracted by water or causing the formation of an emulsion. Since fuels such as gasolines are almost always brought into contact with water, either intentionally or unintentionally, a high level of water interaction is undesirable.

3. With respect to the phosphorus-containing anti-icing additives, the presence of phosphorus in the fuel may undesirably affect the operation of a catalytic muffler or thermal reactor which is connected to the engine to control exhaust emissions, for example, hydrocarbons, carbon monoxide and oxides of nitrogen.

Combinations or mixtures of compounds which are disclosed in the art as anti-icing or anti-stalling additives for gasoline include the following. British 997,906 discloses gasolines which have anti-icing characteristics and contain 0.02-0.05% by volume of (a) two or more gasoline soluble diols which are addition products derived from 1 to 3 moles of 1,2-propylene oxide and 1

5 mole of propanediol-1,2; (b) two or more gasoline soluble alkylene glycol ethers of the formula  $R-(OCH_2CH_2)_n-OH$  wherein R is  $C_{1-4}$  alkyl and n is 2 or 3; or (c) a mixture of one or more diols of (a) and one or more ethers of (b). U.S. Pat. No. 3,336,123 discloses gasolines containing as an anti-stalling agent an effective amount of a salt of a linoleic acid dimer or trimer and a dialkylaminopropyl-carboxamide of the formula 10  $Ac-NH-CH_2CH_2CH_2-NRR'$  wherein Ac is a  $C_{8-18}$  fatty or naphthyl acyl group and R and R' are the same or different and are  $C_{1-4}$  alkyl groups. It also discloses that neither the acid nor the amine components of the salt exhibit anti-icing characteristics. U.S. Pat. No. 3,647,378 discloses gasolines which have improved 15 anti-icing properties and which contain a mixture of benzoic acid and a surfactant type deicer, such as oleyl amine, or a freeze-point depressant type deicer, such as a glycol ether. U.S. Pat. No. 3,653,853 discloses a synergistic anti-icing composition for gasoline, which composition contains a polyhydroxy aliphatic alcohol of 2-8 carbon atoms and a  $C_{8-20}$  aliphatic amide of a  $C_{8-20}$  alkylene diamine, the amount of alcohol being 0.5-5 weight % of the amide. U.S. Pat. No. 3,687,644 discloses 20 gasolines containing as anti-icing additives 0.00001-0.02 weight % of a mono- or polycarboxylic acid, or an anhydride, ester, amide or imide derivative thereof, and 0.01-5 weight % of an alcohol, glycol or polyol.

## SUMMARY OF THE INVENTION

It is an object of the present invention to provide an effective anti-icing gasoline additive composition. It is a further object of the invention to provide an effective, 35 gasoline soluble anti-icing composition which is economical and commercially feasible and which, in addition, provides good anti-rust protection and water interaction properties and is free of any component which may be harmful to exhaust emission control devices. In summary, the present invention resides in a gasoline soluble anti-icing composition which comprises 30-90 weight % of a gasoline soluble organic compound of the formula  $Z-OH$  and 10-70 weight % of a gasoline soluble polycarboxy hydrocarbon having 40 25-75 carbon atoms and at least ten carbon atoms per carboxy group, Z containing about 4-180 carbon atoms and being selected from aliphatic hydrocarbyl, hydroxylaliphatic hydrocarbyl, hydro-poly(oxyalkylene), alkyl poly(oxyalkylene) and alkylphenyl poly(oxyalkylene). Preferred compounds having the formula  $Z-OH$  include compounds of the formulas  $ROH$ ,  $HOR^1OH$  and  $R^2(OH^3)_nOH$  wherein R is  $C_{4-18}$  alkyl,  $R^1$  is  $C_{6-10}$  alkylene,  $R^2$  is H,  $C_{1-18}$  alkyl or  $C_{1-12}$  alkyl(phenyl),  $OR^3$  is  $OCH_2CH_2$ ,  $OCH_2CH_2CH_2$  or  $OCH_2CHCH_3$ , n is 2-60 and any two adjacent  $OR^3$  groups are the same or different. The present invention 50 also resides in gasoline containing the aforesaid anti-icing composition.

## BRIEF DESCRIPTION OF THE DRAWING

The FIGURE includes graphs of  $\Delta$  cycles to stall (a measure of the effectiveness of the additive in gasoline) vs. concentration of the additive in gasoline for the 65 composition of this invention, for each of the individual components of the composition and for the composition of this invention as anticipated (based upon the effectiveness of each individual component).

## DETAILED DESCRIPTION OF THE INVENTION

The present invention resides in the discovery of a composition which is useful as a gasoline anti-icing additive. It also resides in gasoline containing such an additive. The composition of the invention is defined above.

The organic hydroxyl compounds of the composition of this invention are gasoline soluble compounds. Since the present composition is required only in very small amounts in gasoline to impart anti-icing characteristics thereto, by gasoline soluble is meant a solubility of at least about 0.002% by weight in gasoline. The useful organic hydroxyl compounds are represented by the formula Z—OH and include the following:

a. monoalcohols of 4-18 carbon atoms, including both saturated and unsaturated monoalcohols, wherein Z in Z—OH represents an aliphatic hydrocarbyl group of 4-18 carbon atoms. Representative (but non-limiting) examples of Z—OH wherein Z is an aliphatic hydrocarbyl group of 4-18 carbon atoms include butanols, n-octanol, iso-octanol, decanols, decenols, dodecanols, dodecenols, tetradecanols, tetradecenols, hexadecanols, hexadecenols, octadecanols and octadecenols. The alcohols of 8-18 carbon atoms are readily available from vegetable oil, beef tallow and whale oil as well as from synthetic sources such as by the oxo-process and the ethylene telomerization process. The preferred monoalcohols are those produced by ethylene telomerization, such alcohols being commercially available generally as mixtures of straight chain saturated alcohols, such as a mixture which typically contains 1% C<sub>10</sub>H<sub>21</sub>OH, 61% C<sub>12</sub>H<sub>25</sub>OH, 26% C<sub>14</sub>H<sub>29</sub>OH, 11% C<sub>16</sub>H<sub>33</sub>OH and 1% C<sub>18</sub>H<sub>37</sub>OH. For convenience, this mixture will hereinafter be designated as R<sub>12-16</sub>OH.

b. glycols of 6-10 carbon atoms, wherein Z in Z—OH represents a hydroxyaliphatic hydrocarbyl group of 6-10 carbon atoms. Examples include 2,6-hexanediol, 2,5-hexanediol, 1,6-heptanediol, 2,8-octanediol, 2,7-octanediol, 1,8-octanediol, 2,9-decanediol, 2,10-decanediol and 1,10-decanediol.

c. polyoxyalkylene glycols, wherein Z in Z—OH is a hydro-poly(oxyalkylene) group having 6-180 carbon atoms, which can be more simply represented by the formula H(OR<sup>3</sup>)<sub>n</sub>OH wherein R<sup>3</sup> is an alkylene group of 2-3 carbon atoms and n is 2-60, preferably 2-20. These glycols can contain oxyalkylene groups of 2 carbon atoms, oxyalkylene groups of 3 carbon atoms, or both. If the latter, they can be present either in a random distribution or in a block distribution. Such glycols are commercially available. The preferred glycols have oxyalkylene groups wherein the alkylene moiety has 3 carbon atoms and is either a 1,3-propylene or a 1,2-propylene moiety. The preferred compounds are, therefore, H(OCH<sub>2</sub>CH<sub>2</sub>CH<sub>2</sub>)<sub>n</sub>—OH and



wherein n is 2-60, preferably 2-20. It is to be understood that since polyoxyalkylene glycols generally are prepared by the polymerization of alkylene oxides, the value of n will be an average value. Included in this group of polyoxyalkylene glycols are addition products of multifunctional hydroxyl compounds and 1,2-pro-

pylene oxide. Representative of such addition products are



derived from the oxide and trimethylol propane, and



derived from the oxide and pentaerythritol, wherein a and b are such that the total number of carbon atoms is about 15-60.

d. monoalkyl ethers of the polyoxyalkylene glycols of (c). Such alkyl ethers are included in the generic formula previously given, namely, R<sup>2</sup>(OR<sup>3</sup>)<sub>n</sub>OH. R<sup>2</sup> in the formula for such ethers is C<sub>1-18</sub> alkyl (preferably C<sub>12-18</sub> alkyl). Preferred ethers can be represented by the formula



wherein R<sup>4</sup> is an alkyl group of 1-18, preferably 12-18, carbon atoms, j and k are integers, j+k is 7-12, k is 0-4 and j/k is at least 2. The monoalkyl ethers can be prepared by the addition of an alcohol R<sup>4</sup>OH wherein R<sup>4</sup> is an alkyl group of 1-18 carbon atoms to 1,2-propylene oxide followed, if desired, by addition to ethylene oxide, by procedures well known in the art. Although highly purified individual alcohols of 1-18 carbon atoms can be used, it is preferable to use the commercially available mixtures of alcohols discussed above because of their availability and cost. For example, R<sub>12-16</sub>OH, 1,2-propylene oxide and ethylene oxide react to provide an addition product which can be represented by the formula



wherein j and k are as defined above. When both propylene oxide and ethylene oxide are used to prepare the addition product, it is preferred that the ratio of propylene oxide to ethylene oxide in the product be equal to or greater than 2. As an example where the ratio is 2, employing the above formula, j is 8 and k is 4. When only 1,2-propylene oxide is used, that is, k is 0, preferably j is 7-12, more preferably 7.

e. mono(alkylphenyl)ethers of the polyoxyalkylene glycols of (c). They are analogous to the alkyl ethers of (d) and are prepared by the addition of a monoalkylphenol to an alkylene oxide. Such mono(alkylphenyl)ethers are included in the generic formula previously given, namely, R<sup>2</sup>(OR<sup>3</sup>)<sub>n</sub>OH, R<sup>3</sup> being as previously described and R<sup>2</sup> being C<sub>1-12</sub> alkyl(phenyl). Monoalkylphenols are commercially available and are readily prepared by the alkylation of phenol with olefins such as propylene, isobutylene and propylene/isobutylene oligomers. The mono(alkylphenyl)ethers are also commercially available.

The second component of the composition of this invention is a gasoline soluble polycarboxy hydrocarbon

having 25-75 carbon atoms and at least 10 carbon atoms per carboxy group. This acid component of the composition can be represented by the formula  $R^5(COOH)_m$ , wherein  $m$  is 2-5, preferably 2-3, and the number of carbon atoms and the ratio of carbon atoms to carboxy groups are as stated above.  $R^5$  in the formula can be aliphatic, arylaliphatic (preferably phenylaliphatic), cycloaliphatic or arylcycloaliphatic (preferably phenylcycloaliphatic). A readily available polycarboxy hydrocarbon is a dimer-trimer acid. Dimer-trimer acids are well known in the art, for example, as represented by U.S. Pat. No. 2,632,695 and Goebel, Journal of the American Oil Chemists' Society, 24, March, 1947, pages 65-68. Dimer-trimer acids can be produced by the dimerization-trimerization of an unsaturated monocarboxylic acid having, for example, 16-18 carbon atoms, such as by heating an appropriate di- or tri-unsaturated aliphatic carboxylic acid at 330°-360°C. for 3-8 hours in the presence of a small amount of water. Dimer-trimer acids are actually mixtures of dimer acid, which is believed to contain one or more hydroaromatic ring structures, and trimer acid, which is believed to contain two or more hydroaromatic ring structures. A dimer acid is a dibasic or dicarboxylic acid and a trimer acid is a tribasic or tri-carboxylic acid. In carrying out the aforesaid dimerization-trimerization process in a practical fashion, it is difficult to avoid formation of both dimers and trimers. However, by adjusting conditions, such a process can be carried out so as to favor the formation of one or the other acid. For example, under milder conditions, the formation of dimer acid will be favored, in which case the product also usually will contain some unreacted unsaturated acid. Under more rigorous conditions, for example, at higher temperatures and/or heating times, the formation of trimer acid will be favored and essentially 100% conversion of starting unsaturated acid can be achieved. Under such conditions, however, a polymerization type reaction is facilitated and n-mers higher than trimer acid are produced, for example, a tetramer acid. The preferred dimer-trimer acid is derived from linoleic acid. The dimer acid fraction thereof is a dibasic acid containing 36 carbon atoms and the trimer acid fraction thereof is a trimer acid containing 54 carbon atoms. Commercially available linoleic acid dimer acids typically contain about 45-95 wt. % of the dimer acid, about 4-25 wt. % of higher-polymerized linoleic acids and about 0-4 wt. % of monomeric linoleic acid. Commercially available trimer acids typically contain about 75 wt. % of the trimer acid and about 25 wt. % of the dimer acid and the higher-polymerized acids. Other commercially available materials which are suitable herein include dimerized-trimerized tall oil residues which typically contain 30-45 wt. % of dimer acid, 10-30 wt. % of trimer acid, 0-15 wt. % of monocarboxylic acid and 0-20 weight % of rosin acids. "Dimertrimer acid" as the term is employed herein is defined as a composition which contains at least 45 wt. % of dimer and trimer acids, preferably at least 75 wt. % of dimer and trimer acids. Included in the definition are compositions which are comprised substantially of dimer acid and compositions which are comprised substantially of trimer acid.

As already indicated above, the composition of this invention contains about 30-90 wt. % of a gasoline soluble organic hydroxyl compound and about 10-70 wt. % of a polycarboxy hydrocarbon. The choice of a particular ratio of the hydroxyl compound to the acid will

depend upon the hydroxyl compound and acid chosen and the degree of anti-icing protection desired. Other factors may be taken into consideration in choosing a ratio (as will be obvious from the examples), such as 5 water interaction, anti-rust protection and carburetor keep-clean. The preferred composition of this invention comprises about 30-50 wt. % of an organic hydroxyl compound of the formula

10



and about 50-70 wt. % of a dimer-trimer acid derived 15 from linoleic acid since it provides the best overall combination of anti-icing protection, water interaction, anti-rust protection and carburetor keep-clean. The most preferred composition contains 33-34 wt. % of the hydroxyl compound and 66-67 wt. % of the dimer-trimer acid.

20 As noted above, gasoline containing the composition of this invention not only provides excellent carburetor anti-icing protection but it provides excellent water interaction, anti-rust and carburetor keep-clean properties. In addition, since the components of the composition are compounds which contain only carbon, hydrogen and oxygen, the composition does not contain any element which is known to be detrimental to maximum 25 performance of exhaust emission control devices which 30 may be attached to engines operated with such gasolines.

The amount of the composition of this invention which is added to gasoline will depend upon the particular components used in the composition, the nature of 35 the gasoline and the degree of anti-icing protection desired. For example, winter grade gasolines vary in their volatiles content and those which are higher in volatiles content are more apt to produce carburetor icing. Hence, for such gasolines larger amounts of the anti-icing composition are required. With the composition 40 of this invention, anti-icing characteristics have been imparted to gasolines having a 50% distillation point within the range 170°-215°C. (according to ASTM Method D-86) by employing 5 pounds of the composition 45 per 1,000 barrels of gasoline (0.002 wt. %). Preferred amounts of the composition of this invention are in the range 10-20 pounds per 1,000 barrels of gasoline (0.004-0.008 wt. %). The following examples include tests demonstrating the effectiveness of the composition 50 at a use concentration of about 12 pounds per 1,000 barrels of gasoline (1 barrel of gasoline contains 42 gallons). One pound per 1,000 barrels of gasoline is approximately 4 parts per million or 0.0004 wt. %. Higher treating levels, for example, as high as 50-70 55 pounds per 1,000 barrels of gasoline can be used (0.02-0.028 wt. %); however, since the composition of this invention is effective at low concentrations, such higher concentrations merely increase the cost of treatment without providing additional anti-icing benefits.

60 The composition can be added to gasoline in any conventional manner, for example, as a physical mixture of the components or as a 50-90 wt. % concentrate in a solvent such as benzene, toluene or a xylene. The components of the composition can also be added to the 65 gasoline individually if desired. The gasoline to which the composition is added may consist of straight chain or branched chain paraffins, cycloparaffins, olefins and aromatic compounds, or any mixture of these hydro-

carbons, such hydrocarbons being obtainable from straight run naphtha, polymer gasoline, natural gasoline, thermally or catalytically cracked hydrocarbons and catalytically reformed stock. The gasoline may also contain any of the conventional additives, such as tetraalkylead antiknock compounds, halogen-containing scavenging agents, corrosion inhibitors, dyes, antioxidants, anti-rust agents, ether anti-icing agents, gum inhibitors, metal deactivators and anti-pre-ignition agents.

### EXAMPLE 1

This example illustrates the anti-icing properties of the composition of this invention. The anti-icing properties were determined by adding the desired amount of the composition to gasoline and using the gasoline in the Engine Carburetor Anti-icing Test described below. The test is carried out by using a Chevrolet 230 cubic inch, 6 cylinder engine. The environment of the carburetor is maintained at 40°F. and 95% relative humidity. Thus, essentially water saturated cool air is drawn through the carburetor. The test consists of running the engine on a two part cycle, namely, 20 seconds with open throttle at an engine speed of 1,600 r.p.m. and 10 seconds with the throttle almost closed at 400 r.p.m. (idling speed). During the test, ice forms on the throttle plate and on the surrounding carburetor walls and causes the engine to stall by blocking the flow of air

when the throttle plate is almost closed during the idling portion of the test. The base gasoline is chosen so that, normally, in the absence of an effective anti-icing additive, engine stalling occurs after about 3-5 cycles.

5 Generally, an additive is considered to be an effective anti-icing agent if it prevents stalling to about 10 cycles; an excellent anti-icing agent prevents stalling to at least about 25 cycles. The base gasoline used herein had a 10 50% distillation point of 197°F. according to ASTM Method D-86.

The results of this example are summarized in Table I. In the table, the control valve, that is, the number of cycles of stall when gasoline without any additive is used, is recorded as 5, the maximum value obtained in 15 a series of tests. The improvement in anti-icing is the difference between the number of cycles to stall for the gasoline containing the anti-icing agent and the control gasoline ( $\Delta$  cycles to stall). The expected increase in the number of cycles to stall ( $\Delta$  cycles to stall, expected) is the expected increase in the number of cycles to stall based on the amounts of hydroxyl compound and the dimer-trimer acid added to the gasoline, that is, the expected increase due to the cumulative 20 independent effects of the individual components of the composition. The difference between the actual increase and the expected increase demonstrates the synergistic interaction of the components of the composition. 25

TABLE I

| Test No.                                                                                                                                                                    | Acid lb./1,000 bbl. | Hydroxyl Compound lb./1,000 bbl. | Wt. % Hydroxyl Compound | Cycles to Stall | $\Delta$ Cycles to Stall, Expected | $\Delta$ Cycles to Stall |
|-----------------------------------------------------------------------------------------------------------------------------------------------------------------------------|---------------------|----------------------------------|-------------------------|-----------------|------------------------------------|--------------------------|
| I. Control                                                                                                                                                                  |                     |                                  |                         |                 |                                    |                          |
| 1                                                                                                                                                                           | 0                   | 0                                | —                       | 5               | —                                  | —                        |
| 2                                                                                                                                                                           | 5                   | 0                                | 0                       | 6               | —                                  | 1                        |
| 3                                                                                                                                                                           | 12                  | 0                                | 0                       | 7               | —                                  | 2                        |
| 4                                                                                                                                                                           | 17                  | 0                                | 0                       | 11              | —                                  | 6                        |
| 5                                                                                                                                                                           | 20                  | 0                                | 0                       | 25+             | —                                  | 20+                      |
| 6                                                                                                                                                                           | 0                   | 10                               | 100                     | 8               | —                                  | 3                        |
| 7                                                                                                                                                                           | 0                   | 15                               | 100                     | 13              | —                                  | 8                        |
| 8                                                                                                                                                                           | 0                   | 17.5                             | 100                     | 25+             | —                                  | 20+                      |
| 9                                                                                                                                                                           | 1.6                 | 12.4                             | 87.5                    | 9               | 6                                  | 4                        |
| 10                                                                                                                                                                          | 2                   | 15                               | 88.2                    | 25+             | 8                                  | 20+                      |
| 11                                                                                                                                                                          | 4                   | 8                                | 67                      | 10              | 4                                  | 5                        |
| 12                                                                                                                                                                          | 5                   | 10                               | 67                      | 25+             | 4                                  | 20+                      |
| 13                                                                                                                                                                          | 6                   | 6                                | 50                      | 12              | 5                                  | 7                        |
| 14                                                                                                                                                                          | 7                   | 7                                | 50                      | 25+             | 4                                  | 20+                      |
| 15                                                                                                                                                                          | 8                   | 4                                | 33                      | 12              | 3                                  | 7                        |
| 16                                                                                                                                                                          | 9                   | 5                                | 35                      | 25+             | 4                                  | 20+                      |
| II. Acid = Dimer-Trimer Acid <sup>(1)</sup> Hydroxyl Compound = R <sub>12-16</sub> —(OCH <sub>2</sub> —CH) <sub>n</sub> —OH                                                 |                     |                                  |                         |                 |                                    |                          |
| 17                                                                                                                                                                          | 0                   | 8.75                             | 100                     | 8               | —                                  | 3                        |
| 18                                                                                                                                                                          | 7.5                 | 7.5                              | 50                      | 16              | 4                                  | 11                       |
| 19                                                                                                                                                                          | 8.75                | 8.75                             | 50                      | 25+             | 4                                  | 20+                      |
| III. Acid = Dimer-Trimer Acid <sup>(1)</sup> Hydroxyl Compound = H(OCH <sub>2</sub> CH) <sub>12</sub> —OH                                                                   |                     |                                  |                         |                 |                                    |                          |
| 20                                                                                                                                                                          | 0                   | 10                               | 100                     | 10              | —                                  | 5                        |
| 21                                                                                                                                                                          | 5                   | 10                               | 67                      | 25+             | 6                                  | 20+                      |
| 22                                                                                                                                                                          | 7.5                 | 7.5                              | 50                      | 14              | 6                                  | 9                        |
| 23                                                                                                                                                                          | 8.75                | 8.75                             | 50                      | 25+             | 6                                  | 20+                      |
| 24                                                                                                                                                                          | 10                  | 5                                | 33                      | 25+             | 6                                  | 20+                      |
| IV. Acid = Dimer-Trimer Acid <sup>(1)</sup> Hydroxyl Compound = R <sub>12-16</sub> (OCH <sub>2</sub> CH) <sub>n</sub> —(OCH <sub>2</sub> CH <sub>2</sub> ) <sub>4</sub> —OH |                     |                                  |                         |                 |                                    |                          |
| 25                                                                                                                                                                          | 0                   | 8.75                             | 100                     | 8               | —                                  | 3                        |
| 26                                                                                                                                                                          | 7.5                 | 7.5                              | 50                      | 9               | 4                                  | 4                        |
| 27                                                                                                                                                                          | 8.75                | 8.75                             | 50                      | 25+             | 4                                  | 20+                      |
| V. Acid = Dimer-Trimer Acid <sup>(1)</sup> Hydroxyl Compound = H(OCH <sub>2</sub> CH) <sub>12</sub> —OH                                                                     |                     |                                  |                         |                 |                                    |                          |
| 28                                                                                                                                                                          | 0                   | 8.75                             | 100                     | 8               | —                                  | 3                        |
| 29                                                                                                                                                                          | 7.5                 | 7.5                              | 50                      | 10              | 4                                  | 5                        |
| 30                                                                                                                                                                          | 8.75                | 8.75                             | 50                      | 25+             | 4                                  | 20+                      |
| VI. Acid = Dimer-Trimer Acid <sup>(1)</sup> Hydroxyl Compound = Dipropylene Glycol                                                                                          |                     |                                  |                         |                 |                                    |                          |
| 31                                                                                                                                                                          | 0                   | 10                               | 100                     | 6               | —                                  | 1                        |
| 32                                                                                                                                                                          | 8.75                | 8.75                             | 50                      | 13              | 2                                  | 8                        |
| 33                                                                                                                                                                          | 10                  | 10                               | 50                      | 25+             | 3                                  | 20+                      |

TABLE I-continued

| Test No.                                                                                                                                  | Acid lb./1,000 bbl. | Hydroxyl Compound lb./1,000 bbl. | Wt. % Hydroxyl Compound | Cycles to Stall | ΔCycles to Stall, Expected | ΔCycles to Stall |
|-------------------------------------------------------------------------------------------------------------------------------------------|---------------------|----------------------------------|-------------------------|-----------------|----------------------------|------------------|
| I. Control                                                                                                                                |                     |                                  |                         |                 |                            |                  |
| VIII. Acid = Dimer-Trimer Acid <sup>(1)</sup> Hydroxyl Compound = 2,5-Hexanediol                                                          |                     |                                  |                         |                 |                            |                  |
| 34 0                                                                                                                                      | 10                  | 100                              | 9                       | —               | 4                          |                  |
| 35 5                                                                                                                                      | 10                  | 67                               | 25+                     | 5               | 20+                        |                  |
| 36 7.5                                                                                                                                    | 7.5                 | 50                               | 9                       | 5               | 4                          |                  |
| 37 8.75                                                                                                                                   | 8.75                | 50                               | 25+                     | 5               | 20+                        |                  |
| 38 10                                                                                                                                     | 5                   | 33                               | 25+                     | 6               | 20+                        |                  |
| IX. Acid = Dimer-Trimer Acid <sup>(1)</sup> Hydroxyl Compound = Iso-octylphenol/ethylene oxide Addition Product                           |                     |                                  |                         |                 |                            |                  |
| 39 0                                                                                                                                      | 10                  | 100                              | 9                       | —               | 4                          |                  |
| 40 8.75                                                                                                                                   | 8.75                | 50                               | 15                      | 5               | 10                         |                  |
| 41 10                                                                                                                                     | 10                  | 50                               | 25+                     | 7               | 25+                        |                  |
| X. Acid = Dimer-Trimer Acid <sup>(1)</sup> Hydroxyl Compound = Oxo-Decyl Alcohol                                                          |                     |                                  |                         |                 |                            |                  |
| 42 0                                                                                                                                      | 30.0                | 100                              | 14                      | —               | 9                          |                  |
| 43 7.5                                                                                                                                    | 7.5                 | 50                               | 11                      | 4               | 6                          |                  |
| 44 8.75                                                                                                                                   | 8.75                | 50                               | 25+                     | 4               | 20+                        |                  |
| XI. Acid = Dimer-Trimer Acid <sup>(2)</sup> Hydroxyl Compound = R <sub>12-16</sub> —(OCH <sub>2</sub> —CH <sub>2</sub> ) <sub>7</sub> —OH |                     |                                  |                         |                 |                            |                  |
| 45 20 0                                                                                                                                   | 0                   | 0                                | 7                       | —               | 2                          |                  |
| 46 12.5 12.5                                                                                                                              | 12.5                | 50                               | 13                      | 6               | 8                          |                  |
| XII. Acid = Dimer-Trimer Acid <sup>(3)</sup> Hydroxyl Compound = R <sub>12-16</sub> —(OCH <sub>2</sub> CH <sub>2</sub> ) <sub>7</sub> —OH |                     |                                  |                         |                 |                            |                  |
| 47 20 0                                                                                                                                   | 0                   | 0                                | 5                       | —               | 0                          |                  |
| 48 10 10                                                                                                                                  | 50                  | 25+                              | 3                       | 20+             |                            |                  |

<sup>(1)</sup>Dimer-Trimer Acid = C<sub>20</sub> dibasic acid (45%); C<sub>18</sub> monobasic acid (13%); C<sub>16</sub> tribasic and higher acids (25%); rosin acids (14%); residual (3%)

<sup>(2)</sup>Dimer-Trimer Acid = C<sub>20</sub> dibasic acid (75%); C<sub>18</sub> tribasic acid (25%); C<sub>16</sub> monobasic acid (trace)

<sup>(3)</sup>Dimer-Trimer Acid = C<sub>18</sub> tribasic acid (90%); C<sub>20</sub> dibasic acid (10%)

The above data clearly show that the composition of this invention provides better anti-icing protection than would be expected on the basis of the expected contribution of each of the components of the combination. The synergistic anti-icing activity of the combination also is obvious from the FIGURE which is a plot of Δ cycles to stall vs. concentration of additive. The FIGURE shows the improvement in anti-icing provided by Dimer-Trimer Acid<sup>(1)</sup> (Curve A) and by



These curves are based on the data of test numbers 1-8 in Table I. Curve C represents the anti-icing improvement to be expected upon combination of equal weights of Dimer-Trimer Acid<sup>(1)</sup> and hydroxyl compound. Curve D represents the actual anti-icing improvement obtained with a composition containing equal weights of Dimer-Trimer Acid<sup>(1)</sup> and hydroxyl compound as shown by test numbers 13 and 14 in Table I. It can be seen from Curve D that the composition containing 7 pounds per 1,000 barrels of the Dimer-Trimer Acid<sup>(1)</sup> and 7 pounds per 1,000 barrels of hydroxyl compound gave excellent anti-icing improvement of Δ cycles to stall of 20+ whereas from Curve C it would be expected that the composition should contain 17 pounds per 1,000 barrels each of the Dimer-Trimer Acid<sup>(1)</sup> and hydroxyl compound to give the same Δ cycles to stall of 20+. Similar curves can be drawn from the data summarized in Table I for other ratios of the hydroxyl compound to Dimer-Trimer Acid<sup>(1)</sup> as well as for other compositions and components to show that similar types of synergistic anti-icing improvements were obtained.

## EXAMPLE 2

This example illustrates that the composition of the invention, when incorporated into gasoline, in addition to providing excellent anti-icing protection, also provides excellent anti-rust, carburetor keep-clean and water interaction properties. The composition used was a combination of 67% of Dimer-Trimer Acid<sup>(1)</sup> and 33% of



The composition was added to the gasoline at a treating level of 14 pounds per 1,000 barrels. Rust-preventing characteristics of the treated gasoline were determined according to ASTM Method D665 Procedure A. A mixture of 300 ml. of gasoline and 30 ml. of distilled water, at a temperature of 140°F., was stirred with a cylindrical steel specimen completely immersed therein. The test was run for 24 hours and the area of rust on the specimen was reported as % rust. The carburetor keep-clean test (Onan) was carried out in a single cylinder engine to which a controlled amount of exhaust gas from another engine was mixed with air supplied to the test carburetor. The test carburetor throat consisted of a two-piece stainless steel liner fitted around the throttle plate shaft. The liner was easily removed for inspection and rating. The engine was operated under cycling conditions of one minute idling and three minutes part throttle for an overall test period of 2 hours. A visual rating scale of 10 for a clean carburetor and 0 for a very dirty one was used. Generally, a rating of 6 or greater is considered as satisfactory carburetor keep-clean. Water interaction properties of the gasoline containing the composition of the invention were determined by the United States Federal Water Contact Test, Test Method Standard 791B - Method

## 11

3251.7. The fuel to be tested (80 ml.) was shaken with 20 ml. of a phosphate buffer and after standing for 5 minutes the change in the volume of the aqueous layer and the condition of the interface between the two layers were noted. The interface condition was rated as follows: (1) clear clean interface; (1b) a few small clear bubbles covering not more than estimated 50% of the interface and no shreds, lace and/or film at the interface; (2) shred of lace and/or film at interface; (3) loose lace and/or slight scum; and (4) tight lace and/or heavy scum. For the water interaction test, the anti-icing composition was added to the gasoline at a level of 50 pounds per 1,000 barrels. The results of the tests are summarized below.

TABLE II

| Tests                                        | Control Gasoline | Anti-icing Composition 14 lbs./1,000 bbl. |
|----------------------------------------------|------------------|-------------------------------------------|
| 1. % Rust ASTM D665 A                        | 80               | 0                                         |
| 2. Carburetor Keep-Clean (Onan)              | 4.5              | 7.8                                       |
| 3. Water Interaction Fed. Test Method 3251.7 | 1                | 1 <sup>10</sup>                           |
| 4. Anti-icing, Cycles to Stall               | 3-5              | 25+                                       |

<sup>10</sup>Anti-icing composition at 50 lbs./1,000 bbl.

The above data clearly show that the composition of this invention, in addition to providing good anti-icing protection at low concentrations (14 lbs./1,000 bbl.), also provides good anti-rust protection, good carburetor keepclean and good water interaction properties. As shown in Table II, water interaction tests carried out with 50 pounds of additive per 1,000 barrels of gasoline gave an interface rating of 1; hence, it is apparent that at lower treating levels, the rating will be equally as good.

The embodiments of the invention in which an exclusive property or privilege is claimed are defined as follows:

1. An anti-icing composition for gasoline and comprising 30-90 weight % of a gasoline soluble organic compound of the formula Z—OH and 10-70 weight % of a gasoline soluble dimer-trimer acid of a C<sub>16-18</sub> unsaturated, aliphatic monocarboxylic acid, Z—OH being selected from the group consisting of ROH, HOR<sup>1</sup>OH and R<sup>2</sup>(OR<sup>3</sup>)<sub>n</sub>OH wherein R is C<sub>4-18</sub> alkyl, R<sup>1</sup> is C<sub>6-10</sub> alkylene, R<sup>2</sup> is H, C<sub>1-18</sub> alkyl or C<sub>1-12</sub> alkyl(phenyl), R<sup>3</sup> is C<sub>2-3</sub> alkylene, n is 2-60 and any two adjacent OR<sup>3</sup> groups are the same or different.

2. The composition of claim 1 wherein Z—OH is the compound having the formula R<sup>2</sup>(OR<sup>3</sup>)<sub>n</sub>OH wherein R<sup>2</sup>

is H, C<sub>1-18</sub> alkyl or C<sub>1-12</sub> alkyl(phenyl), OR<sup>3</sup> is OCH<sub>2</sub>CH<sub>2</sub>, OCH<sub>2</sub>CH<sub>2</sub>CH<sub>2</sub> or OCH<sub>2</sub>CHCH<sub>3</sub>, n is 2-60 and any two adjacent OR<sup>3</sup> groups are the same or different.

3. The composition of claim 2 wherein R<sup>2</sup> is C<sub>1-18</sub> alkyl.

4. The composition of claim 3 wherein R<sup>2</sup> is C<sub>12-18</sub> alkyl and n is 2-20.

5. The composition of claim 1 wherein Z—OH is the compound having the formula



wherein R<sup>4</sup> is C<sub>12-18</sub> alkyl, j and k are integers, j + k is 7-12, k is 0-4 and j/k is at least 2.

6. The composition of claim 5 wherein j is 8 and k is 4.

7. The composition of claim 5 wherein j is 7-12 and k is 0.

8. The composition of claim 1 wherein Z is C<sub>4-18</sub> alkyl.

9. The composition of claim 1 wherein Z—OH is the compound having the formula H(OR<sup>3</sup>)<sub>n</sub>OH wherein R<sup>3</sup> is C<sub>3</sub> alkylene and n is 2-20.

10. The composition of claim 1 wherein the dimer-trimer acid is substantially dimer acid.

11. The composition of claim 1 wherein the dimer-trimer acid is substantially trimer acid.

12. Gasoline containing an amount of the composition of claim 1 sufficient to impart anti-icing characteristics to the gasoline.

13. The gasoline of claim 12 wherein the composition of claim 1 comprises 0.002-0.02 weight % of the gasoline.

14. The gasoline of claim 13 wherein the composition of claim 1 comprises 0.004-0.008 weight % of the gasoline.

\* \* \* \* \*